

Aug. 23, 1932.

M. S. McCONOUGHY

1,873,844

METHOD OF MAKING LINOLEUM

Filed April 24, 1928



INVENTOR  
Merle S. McConoughey

BY *Gordon C. Willard*  
ATTORNEY

## UNITED STATES PATENT OFFICE

MERLE S. McCONOUGH, OF TUCSON, ARIZONA, ASSIGNOR TO CONGOLEUM-NAIRN, INC.,  
A CORPORATION OF NEW YORK

## METHOD OF MAKING LINOLEUM

Application filed April 24, 1928. Serial No. 272,427.

The present invention relates to the manufacture of sheets of linoleum or the like wherein lump, or granular or other form of plastic linoleum composition is consolidated by means of calendering or sheeting rolls. This application is a continuation in part of my copending application, Serial No. 200,614, filed June 22, 1927, upon which issued Patent No. 1,763,314.

Various primary types of floor coverings that are called linoleum were invented and were named "linoleum" by Walton more than fifty years ago. His original linoleum composition consisted essentially of linoxylinseed oil, resin and kauri gum, especially prepared and combined with filling material such as wood pulp, ground cork or the like, with pigments sometimes added to give the desired color. It is characteristic of these compositions that they are plastic at normal temperature so that they can be rolled to sheet form, and that thereafter they can be cured and oxidized by long continued exposure to hot air, to the elastic firmness characteristic of the finished product. While numerous changes have been proposed in the proportions of the materials used in the linoleum composition, and various additions and substitutions have been made, usually with the view of improving some quality of the product, the essential characteristics of the completed product and of the method of production are today generically the same as they were fifty years ago.

The chief object of the present invention is to provide a novel method for the continuous production, by means of calendering or sheeting rolls, of sheet linoleum from plastic linoleum composition of the generic type described above, but wherein the relative proportion of the costly linoxylinseed oil or cement is materially reduced, thereby effecting a substantial decrease in the cost of the finished product. A further object of my invention is to provide a novel process for the continuous production of sheet linoleum wherein the percentage of imperfect or damaged goods is very substantially decreased, this factor likewise operating to reduce the man-

ufacturing costs. A still further object of my invention comprises the provision of a method whereby unusually attractive decorative effects may be obtained by consolidating vari-colored plastic linoleum compositions by means of calender rolls to produce a variegated pattern wherein the several color areas are sharply defined.

According to the general practice of consolidating plastic linoleum composition by means of calender or sheeting rolls, the plastic material is fed to the sheeting rolls at or slightly above atmospheric temperature. During the consolidating operation a large amount of heat is developed by friction in the material and between the material and the consolidating rolls, causing the temperature of the composition and of the rolls to rise very considerably, say to 125°-175° F. In order to cause the formed sheet to adhere to one roll in preference to the other, cold water is circulated thru the one and steam thru the other, thereby creating a small temperature differential between the two rolls, the formed sheet sticking to the cooler thereof. The maintenance of a small temperature differential in this manner does not, however, serve to provide any positive control of the absolute temperature of the rolls or of the composition, and the temperature of the so-called "cooler" or "sheet carrying" roll may normally be of the order of 125°-150° F., depending on conditions. Thus, under former conditions of continuous operation, or substantially continuous operation, the working of this material develops such large amounts of heat that the peripheral surface of the sheeting roll becomes hot and remains considerably above atmospheric temperatures, even in the case of a "sheet carrying" roll having a central bore through which water is circulated. At such temperatures, even in spite of the small temperature differential between the rolls, the formed sheet has a tendency not to adhere to the cooler roll (or to either roll) but to fall therefrom at intervals and frequently to break, thereby causing delays and damaged goods. To reduce the liability and frequency of these occurrences, the proportion of the costly li-

neum composition of the generic type described above, but wherein the relative proportion of the costly linoxylinseed oil or cement is materially reduced, thereby effecting a substantial decrease in the cost of the finished product. A further object of my invention is to provide a novel process for the continuous production of sheet linoleum wherein the percentage of imperfect or damaged goods is very substantially decreased, this factor likewise operating to reduce the man-

noxyn cement in the linoleum composition is increased very considerably beyond that required for the production of a satisfactory finished product, in order to make the composition more sticky and therefore, more adherent to the sheet carrying roll. But even by adopting this expensive expedient, the difficulties are not wholly avoided, and frequent delays are encountered and imperfect goods produced by failure of the formed linoleum sheet to adhere properly to the sheet carrying roll.

I have discovered that these difficulties may be overcome and the objects and advantages enumerated above may be obtained, if the sheeting rolls, or more particularly the roll which carries the sheet is prevented from heating up to the temperature that naturally results from the heat developed in the consolidating operation, say 125°-150° F., and if such roll be positively cooled to and maintained at approximately atmospheric temperature or below. Broadly, my invention consists in consolidating plastic linoleum composition by means of sheeting or calender rolls, while positively controlling the temperature of the sheet carrying roll to maintain the same at approximately atmospheric temperature, e. g. approximately 70° F., or, and preferably, below, whereby the consolidation of the plastic linoleum composition is accomplished without any substantial rise in temperature.

The above and other features of my invention may be more fully understood from the following description in connection with accompanying drawing in which:

Fig. 1 represents a front view of a machine for sheeting plastic linoleum composition in accordance with my invention, and

Fig. 2 is a sectional elevation taken on the line of 2—2 of Fig. 1.

Fig. 3 is a longitudinal section of the sheet carrying roll.

In the drawing, a pair of sheeting rolls, 1 and 2, rotate in suitable bearings carried by the frame, 3. The rolls are positively driven by any suitable mechanism, conventionally indicated by the pinion, 4, and gear, 5. A hopper or chute, 6, above the rolls, serves to receive the granular, lump or other form of plastic linoleum composition and to convey it to the bite of the rolls. In passing between the rolls, the plastic composition is consolidated by pressure to form a continuous sheet, 7, such consolidation being accompanied by the generation and liberation of a large amount of heat. The sheet, 7, thus formed, will tend to cling to the cooler of the two rolls, 2, commonly termed the "carrying roll", and will be stripped therefrom by a doctor blade, 8, located in a suitable position.

In order to provide for rapid absorption of a large amount of heat and thereby be able to positively control the absolute tem-

perature of the sheet carrying roll, 2, I employ a structure of special design which is capable of rapid heat transfer and is of such structural rigidity as to withstand the enormous physical stresses to which rolls of this type are normally subjected. More particularly the roll, 2, is provided with a plurality of passages, 10, 10', etc., located near the periphery thereof, and communicating with annular chambers 11, 11', at the respective ends of the roll. The chambers, 11, 11', are in communication, respectively, with the inlet, 12, and outlet, 15, by means of the passages 13, 14. Brine or other refrigerating medium, provided from a suitable source, and maintained at low temperature, say 5° to 20° F., is continuously admitted thru the inlet, 12, circulated thru the passages, 10, 10', etc., and removed thru the outlet, 15. In this manner I am able to positively control the temperature of the sheet carrying roll and thereby continuously absorb and remove substantially all of the heat generated in the consolidating operation. Since a small temperature differential between the rolls is required in order to cause the formed linoleum sheet to adhere to one roll in preference to the other, roll 1 will not be maintained at as low a temperature as roll 2, and may normally be of the well known central bore type. However, instead of circulating steam therethru, as has been the practice heretofore, brine or cold water is used to aid in the absorption of heat.

Altho it will not usually be found necessary, additional cooling of the sheet carrying roll may be accomplished by means of an external cooling jacket positioned in heat transfer relation with surface of the roll, a suitable type of jacket being described in my copending application Serial No. 200,615, filed June 22, 1927.

In all events, sufficient refrigeration or cooling of the sheet carrying roll will be employed in order to maintain said roll at approximately atmospheric temperature or below, whereby the plastic linoleum composition is consolidated between the rolls without substantial rise in temperature of the composition. In some cases as for example, where the incoming plastic linoleum composition is relatively warm, it may even be found desirable to cause a reduction in the temperature of the composition during, and simultaneously with, the consolidating operation.

By positively controlling the temperature of the sheet carrying roll, as above indicated, I am able to maintain the formed linoleum sheet strongly adherent to the roll at all times. This avoids the difficulties above set forth, namely, the premature stripping of the sheet from the roll before reaching the doctor blade, which occurrence frequently causes the sheet to break and nearly always

produces a sheet having a rough surface, commonly known in the art as "chatter marks". Furthermore, I am able to employ a linoleum composition in which the relative proportion of the costly linoxyn cement is materially reduced, such less proportion of cement being quite satisfactory for the production of a high quality product, but which amount is insufficient to cause the formed sheet to steadily adhere to a roll whose temperature is of the order of 125° to 150° F. This saving in linoxyn cement together with the saving effected by the marked decrease in the percentage of damaged goods, very substantially reduces the cost of the ultimate product.

My invention also enables the production of unusually attractive decorative effects when consolidating vari-colored linoleum composition, by reason of the fact that the relatively low temperature of the linoleum composition and sheet carrying roll during the consolidating operation, prevents any substantial smearing or blending of the several colors, particularly when the rolls are rotated at approximately the same speed. In this manner I am able to obtain a variegated pattern wherein the several color areas are sharply defined.

An advantage inherent in the rolling of linoleum composition in accordance with this invention is that a gummy film does not form on rolls by which linoleum composition is treated and which are cooled in accordance with this invention, whereas such a film forms on rolls not so cooled and accumulates on the edge of a doctor blade used to strip the sheet of composition from the roll. The accumulated gum on the edge of the blade injures and breaks the sheet and requires shutting down of the sheeting operation for its removal.

From the foregoing it is apparent that in the practice of this invention linoleum composition may be rolled in accordance with the prior procedures involving either rolling the composition into an unbacked sheet which is subsequently applied to a backing material or rolling the composition directly upon the backing material; and it is also apparent that the composition employed may be from any source and may be of a single color or composed of composition of different colors and may be composed of granules or lumps which may or may not be of different colors. Moreover, the mass of linoleum composition may be either wholly unformed or may have already been formed into formed masses such as sheets, and such sheets may have been placed in overlapping relation. For example, as in Patent No. 1,763,814, above mentioned, which issued on the application of which this application is a continuation in part, the mass of linoleum composition may comprise masses such as lumps or granules of dif-

ferent colors, and such mass may be rolled in one direction into sheets in which the different colors appear as striations extending in the direction in which the rolling occurred, and the resulting mass comprising said sheets is subsequently subjected to cross rolling as by maintaining a continuous supply of said sheets overlapped transversely to the striations caused by the first rolling. In such case the maintaining of the periphery, of that roll of the cross rollers which contacts with the face of the resulting sheet, at or below a temperature at which undesirable smearing of the composition and blending of the colors occurs, e. g. at a temperature not substantially above and preferably below atmospheric temperature, according to this invention, affords a beautiful marble effect in which the colored portions are not smeared upon one another but are clearly defined.

As will be apparent to those skilled in the art, this invention contributes an important advance in the linoleum industry in that it teaches for the first time a method of sheeting linoleum composition under conditions of temperature discovered to provide unusual advantages, and which conditions are diametrically opposed to the heretofore accepted theory and practice of the linoleum art. In the teaching of this method and its advantages the present inventor asserts his pioneer-ship.

The calender roll described herein is generically and specifically claimed in a co-pending application Serial No. 272,019 filed April 23, 1928.

I claim:

1. In a method of producing a sheet of linoleum composition wherein a mass of plastic linoleum composition comprising compositions of different colors is introduced and continuously consolidated under pressure between sheeting rolls to produce a sheet of linoleum composition having a variegated design, the step comprising preventing the heat to which the sheeting rolls are subjected during substantially continuous operation over a protracted period of time from increasing the temperature of the periphery of one of the rolls in contact with the linoleum to a temperature in excess of substantially atmospheric temperature.

2. In a method of producing a sheet of linoleum composition wherein a mass of plastic linoleum composition comprising compositions of different colors is introduced and continuously consolidated under pressure between sheeting rolls to produce a sheet of linoleum composition having a variegated design, the step comprising maintaining the temperature of the periphery of one of said rolls, by withdrawing heat from said periphery, below that temperature at which substantial smearing or blending of the different colors will occur, and thereby producing in

the face of the resulting linoleum sheet a variegated design having clearly defined color areas.

3. A process of making sheet linoleum composition which comprises introducing the composition to calender rolls, substantially continuously consolidating the composition between the rolls to form a consolidated sheet and thereby subjecting said rolls for indefinite periods of time to heat generated by work done upon the linoleum composition during said consolidation thereof under pressure between said rolls, and simultaneously circulating a refrigerant adjacent the periphery of one of said calender rolls and while said roll is in direct sheet-forming pressure contact with said composition, thereby maintaining the surface of said roll substantially at or below atmospheric temperature while in direct contact with said composition and during the consolidation of said composition into sheet form.

4. In a process of making a sheet of linoleum composition wherein a mass of linoleum composition composed of compositions of different colors is fed to sheeting rolls and is consolidated between said rolls under pressure to produce a sheet of linoleum composition having a variegated design, the steps comprising subjecting the mass of linoleum composition to a substantially continuous sheeting operation for an indefinite period of time, and simultaneously cooling the surface of one of said rolls and thereby maintaining said surface at approximately atmospheric temperature or below, thereby preventing the smearing or blending of said linoleum compositions of different colors and preserving the definition between the different colors of said design.

5. In a method of rolling linoleum composition containing a drying oil binding material into sheet form between sheeting rolls wherein the sheeting rolls are subjected substantially continuously to heat generated by work done upon the linoleum composition during consolidation thereof under pressure between said sheeting rolls, the steps comprising maintaining substantially at or below atmospheric temperature the periphery of one sheeting roll which is in contact with said linoleum composition and which forms one face of the resulting linoleum sheet, and maintaining the other of said rolls at a substantially higher temperature, and thereby imparting to the sheet increased tensile strength and causing it to adhere to the cooler of said rolls.

6. In a process of making a sheet of linoleum composition wherein a mass of linoleum composition composed of compositions of different colors is fed to sheeting rolls and is consolidated between said rolls under pressure to produce a sheet of linoleum composition having a variegated design, the steps

comprising subjecting the mass of linoleum composition to a substantially continuous sheeting operation for an indefinite period of time, and simultaneously cooling the surface of that sheeting roll which is in contact with said composition and which forms the face of said sheet and thereby maintaining that surface at a temperature below the temperature at which substantial smearing or blending of the linoleum compositions of different colors will occur, to produce in the face of the resulting linoleum sheet a variegated design having clearly defined color areas.

In testimony whereof, I affix my signature.

MERLE S. McCONUGHEY.